

## UNITED STATES PATENT OFFICE

2,341,565

## COMPOUNDED OIL

Arthur L. Lyman, Berkeley, and Lloyd H. Mulin,  
Richmond, Calif., assignors to Standard Oil  
Company of California, San Francisco, Calif., a  
corporation of Delaware

No Drawing. Application January 22, 1940,  
Serial No. 315,034

3 Claims. (Cl. 252—48)

This invention relates to a new and useful composition of matter and involves a composition comprising a hydrocarbon oil and a new combination of stabilizing ingredients. More particularly, the invention pertains to a viscous hydrocarbon oil containing a metal alcoholate and an oxidation inhibitor.

The production of improved hydrocarbon oils, and particularly of lubricating oils having desired characteristics, has been the subject of extensive research. Generally speaking, the compounding of hydrocarbon oils to obtain desired characteristics involves empirical phenomena and the action of untested combinations of different types of compounding agents cannot be predicted.

A characteristic which has been the subject of extensive investigation is the tendency of hydrocarbon oils to deteriorate or partially decompose and oxidize when subjected to high temperatures. This deterioration is evidenced by the deposition of adhesive deposits on hot metal surfaces over which the hydrocarbon oil may flow. It is important that resistance to such deterioration be imparted to hydrocarbon oils, particularly to lubricating oils, in order that such compositions may be relatively free from the tendency to form such deposits even under high temperatures and severe operating conditions. A direct result of this type of deterioration during lubrication of internal combustion engines is the formation of "varnish" on the pistons and cylinder walls, and in engines of the Diesel type a pronounced tendency of the oil to cause or permit the sticking of piston rings.

The crankcase lubricant in internal combustion engines is subjected to extremely severe operating conditions, and in engines of the Diesel type the lubricant encounters in the piston ring zone temperatures of from approximately 425° to 650° F. and pressures from the oxidizing combustion gases as high as 750 to 1150 pounds per square inch. In its more specific aspects the present invention is directed to the improvement of hydrocarbon lubricating oils by imparting thereto increased resistance to deterioration by heat at high temperature levels in the order of those above-mentioned. It has been observed that high temperature oxidation inhibitors, i. e. oxidation inhibitors effective at temperatures as high as 300° F. or above, in combination with metal alcoholates impart to hydrocarbon lubricating oils a number of highly desirable properties and improve the lubrication and operation of internal combustion engines. More particularly, it has been discovered that a lubricating oil containing both a metal alcoholate and a high temperature oxidation inhibitor permits longer periods of op-

eration of engines without the necessity of major overhauls heretofore occasioned by stuck piston rings, wear of pistons and cylinder walls, or in some instances corrosion of bearing metal alloys.

5 The broader aspects of the invention involve the discovery that oxidation inhibitors and metal alcoholates cooperate to give new results in hydrocarbon oil compositions. Hydrocarbon oils containing this combination of ingredients have greater stability under various operating conditions than do oils containing either of these types of ingredients alone. For example, the same improvement is not obtainable with 0.75% of a metal alcoholate or with 0.75% of an antioxidant in a lubricating oil as is obtained with 0.50% of the metal alcoholate and 0.25% of the same antioxidant in the same lubricating oil. Although it has been discovered that oxidation inhibitors in general cooperate with metal alcoholates in the above unpredictable manner, the mechanism of this cooperation has not been established and the inventors therefore refrain from any attempted explanation of the phenomena observed.

20 25 It should be noted that oxidation inhibitors or antioxidants which are effective at low temperatures to inhibit oxidation in hydrocarbon oils may not be effective at higher temperatures and under more severe operating conditions, such as those which lubricating oils encounter in the piston ring belt of internal combustion engines such as Diesel engines. Although the broader aspects of the invention are not so limited, it is preferred to utilize in combination with metal alcoholates high temperature oxidation inhibitors effective above 300° F., and preferably effective to inhibit oxidation of lubricating oils containing metal alcoholates at temperatures in the range of 400° to 500° F.

30 35 40 Metal alcoholates which may be added to hydrocarbon oils, such as mineral lubricating oils, to provide one component of the new composition of matter herein claimed comprise the alkali, alkaline earth, aluminum, and other heavy metal alcoholates. Examples of such alcoholates are: sodium alcoholates, potassium alcoholates, beryllium alcoholates, calcium alcoholates, strontium alcoholates, barium alcoholates, magnesium alcoholates, zinc alcoholates, cadmium alcoholates, and aluminum alcoholates.

45 50 Metal alcoholates which may be utilized and which fall within the scope of this invention are represented by the type formula:

55  $M-(X-C-R)_n$

where M represents a metal, X indicates oxygen or sulfur, C a non-benzenoid carbon atom, R an

organic radical of hydrocarbon structure, and  $n$  is from one to the valence of the metal.  $M$  is a metal such as those previously listed. By "non-benzenoid carbon atom" it is intended to designate a carbon atom which is not in the nucleus of a benzene ring, although attachment to a benzene ring is not precluded. Examples of radicals of hydrocarbon structure which  $R$  represents are: alkyl, aryl, alkaryl, aralkyl and cyclic non-benzenoid.  $R$  need not necessarily be a pure hydrocarbon radical but may contain other substituents, such as oxygen, halogens, nitrogen, and the like. Acyclic radicals are preferred, and the entire compound preferably contains at least ten carbon atoms.

Examples of preferred alcohols utilized to form the metal alcoholate are the higher alcohols, such as amyl, hexyl, heptyl, octyl, nonyl, decyl (lauryl), dodecyl, tetradecyl, hexadecyl (cetyl), octadecyl, ceryl, myricyl, and unsaturated alcohols, such as lanolin alcohol. The following are metal alcoholates of these alcohols which are embraced by this invention: sodium amylate, sodium hexylate, sodium heptylate, sodium octylate, sodium nonylate, sodium decylate, sodium dodecylate, sodium tetradecylate, sodium hexadecylate, sodium octadecylate, sodium cerylate, sodium myricylate, sodium lanolate (sodium salt of lanolin alcohol), calcium amylate, calcium hexylate, calcium heptylate, calcium octylate, calcium nonylate, calcium decylate, calcium dodecylate, calcium tetradecylate, calcium hexadecylate, calcium octadecylate, calcium cerylate, calcium myricylate, calcium lanolate (calcium salt of lanolin alcohol), magnesium amylate, magnesium hexylate, magnesium heptylate, magnesium octylate, magnesium nonylate, magnesium decylate, magnesium dodecylate, magnesium tetradecylate, magnesium hexadecylate, magnesium octadecylate, magnesium cerylate, magnesium myricylate, magnesium lanolate (magnesium salt of lanolin alcohol), barium amylate, barium hexylate, barium heptylate, barium octylate, barium nonylate, barium decylate, barium dodecylate, barium tetradecylate, barium hexadecylate, barium octadecylate, barium cerylate, barium myricylate, barium lanolate (barium salt of lanolin alcohol), aluminum amylate, aluminum hexylate, aluminum heptylate, aluminum octylate, aluminum nonylate, aluminum decylate, aluminum dodecylate, aluminum tetradecylate, aluminum hexadecylate, aluminum octadecylate, aluminum cerylate, aluminum myricylate, and aluminum lanolate (aluminum salt of lanolin alcohol).

Additional alcohols are: cyclo-alkyl alcohols like cyclohexanol, and aralkyl alcohols like benzyl alcohol, as well as acyclic thioalcohols, cyclo-alkyl thioalcohols, and aralkyl thioalcohols, in which sulfur replaces the normal oxygen of the alcoholic group. Examples of thioalcohols are the mercaptans, such as amyl mercaptan, hexyl mercaptan, cyclohexyl mercaptan and the like. Metal derivatives of organic compounds capable of forming the enolic structure also may be utilized. Such derivatives of the enolic compounds contain the group represented by the type formula:



where  $R$  represents an organic radical, preferably a hydrocarbon group, and  $M$  represents a bond to a metal atom.

The metal alcoholates of this invention may be prepared by any suitable method. For example, sodium alcoholates may be prepared by reaction with sodium metal, the calcium alcoholates by reaction of the alcohol with calcium carbide, and the aluminum alcoholates by reaction with metallic aluminum catalyzed with a crystal of iodine.

As has been previously indicated, the invention in its broad aspects embraces hydrocarbon oils containing generically antioxidants for hydrocarbon oils in combination with metal alcoholates. Many antioxidants for hydrocarbon oils are known, and the following types are mentioned for purposes of illustration:

- 15 (1) Oil-soluble hydroxy compounds like polyhydroxy phenols, condensed ring phenols, alkyl substituted phenols, and naturally occurring inhibitors which may be extracted from fats and petroleum oils;
- 20 (2) Nitrogen compounds such as aryl amines (diamines, diaryl amines), nitroso amines, cyclo-aliphatic amines, and condensation products of aldehydes or ketones with aromatic amines;
- 25 (3) Oxygenated organic compounds comprising aryl ethers, aryl ketones and alkyl ketones;
- 30 (4) Esters of certain types of acids, namely, oil-soluble esters of alpha and beta hydroxy carboxylic acids in which a carboxyl group is not more than two carbon atoms removed from a hydroxy group, esters of polycarboxylic acids having two carboxyl groups no more than two carbon atoms apart, and esters of carboxylic acids having an unsaturated carbon-to-carbon bond conjugated with the carboxyl group;
- 35 (5) Oil-soluble organo-metallic compounds of metals selected from groups II, III, IV and V of Mendeleeff's Periodic Table;
- 40 (6) Sulfur, selenium and tellurium compounds (other than compounds in which the sulfur, selenium and tellurium are in a carbocyclic ring), such as aryl mercaptans, sulfides, disulfides, polysulfides, aryl thioesters, seleno ethers, telluro ethers, alkyl sulfides, alkyl disulfides, alkali metal sulfonates, and alkaline earth salts of sulfonic acids;
- 45 (7) Miscellaneous ring compounds comprising mercapto benzothiazole, oxazines, phenothiazine, indane and acridane;
- 50 (8) Organic phosphorus compounds comprising oil-soluble phosphines, esters of phosphorous acid and esters of phosphoric acid;
- 55 (9) Alkaline earth organo-borates and alkaline earth organo-arsenates.

The invention in its more specific aspects involves the combination in hydrocarbon lubricating oils of metal alcoholates and an oxidation inhibitor for the oil effective at temperatures above 300° F. in the presence of the metal alcoholate. Not all of the above-listed antioxidants satisfy this more rigid requirement, and many of them are therefore not fully equivalent to the preferred species utilized in the present invention. Examples of types of high temperature oxidation inhibitors for hydrocarbon oils comprise metal salts of substituted acids of phosphorus, certain oil-soluble esters of carboxylic acids containing an active group, alkali metal sulfonates, alkaline earth metal sulfonates, alkaline earth organo-borates, alkaline earth organo-arsenates, and naturally-occurring inhibitors which may be extracted from mineral oil fractions. By the terms



5  
kyl, or cyclic non-benzenoid radicals. Substituted phosphoric acids containing at least twelve carbon atoms are preferred. Examples of preferred type acids are alkyl or alkaryl substituted phosphoric acids having at least twelve carbon atoms in the molecule. However, it is to be understood that the broader aspects of the invention include other types of substituted oxy-acids of phosphorus containing more than twelve carbon atoms. Additional examples of substituted oxy-acids of phosphorus which may be used in forming the metal salts of the present invention are as follows:



In all of the above formulae R and R' may be 30 alkyl, aryl, alkaryl, aralkyl, or cyclic non-benzenoid groups.

Each and every one of the above antioxidants may be utilized in combination with metal alcoholates in hydrocarbon oils according to the present invention. Hydrocarbon oils containing both a metal alcoholate and an oxidation inhibitor of the above types have new and unpredictable advantages illustrated by the following discussion and data:

A lubricating oil containing a metal alcoholate and a high temperature antioxidant effective above 300° F. in the presence of the alcoholate is more efficient in the lubrication of internal combustion engines than is an oil containing either of the components alone. In engine tests it has been found that metal alcoholates permit the formation of a gum or "varnish" on portions of the pistons after prolonged periods of operation. Various of the metal alcoholates have also been found to impart corrosiveness toward copper-lead or cadmium-silver alloy bearings to lubricating oils containing the same. A high temperature oxidation inhibitor, such as calcium cetyl phosphate, overcomes or minimizes these disadvantages. On the other hand, a calcium cetyl phosphate permits thermal decomposition of the lubricating oil and some deposition of carbon in the top piston ring grooves under severe conditions of operation. The metal alcoholate minimizes this disadvantage of the high temperature oxidation inhibitor. Thus by using these two types of ingredients in combination in lubricating oils, each of which has one or more disadvantages, a lubricating oil having none of the above described objections is obtained and both formation of gum or "varnish" on the piston skirt and deposition of carbon in the piston ring grooves, as well as corrosion of alloy bearings, are prevented or inhibited. The following table gives data illustrating the enhanced effectiveness of the combination in preventing piston ring sticking and in inhibiting "varnish" formation—the piston discoloration number being a measure of "varnish" formation:

| Oil                                                              | Ring sticking | Oil ring clogging 60 hrs. | Piston discoloration number |          |
|------------------------------------------------------------------|---------------|---------------------------|-----------------------------|----------|
|                                                                  |               |                           | 60 hrs.                     | 120 hrs. |
| Acid refined Western oil                                         | Hours         | Percent                   | 1700                        | -----    |
| S. A. E. 30                                                      | 45            | -----                     | -----                       | -----    |
| Ditto + 5% calcium lanolate                                      | 60            | 25                        | 160                         | -----    |
| Ditto + 8% calcium cetyl phosphate                               | 120           | 0                         | 120                         | 225      |
| Ditto + 5% calcium cetyl phosphate + 25% calcium cetyl phosphate | 120+          | 0                         | 70                          | 170      |

<sup>1</sup> Obtained by extrapolation.

15 The following table also gives data establishing the non-corrosiveness of the compounded oil toward copper-lead and cadmium-silver bearing metal alloys, as well as inspections on the used oil showing enhanced stability with the combination of calcium lanolate and calcium cetyl phosphate in the oil:

| Compounding agent               | Acid refined Western oil S. A. E. 30 |                                             |
|---------------------------------|--------------------------------------|---------------------------------------------|
|                                 | None                                 | 0.5% Ca lanolate + 0.25% Ca cetyl phosphate |
| Corrosion—72 hrs. mg. loss:     |                                      |                                             |
| Copper-lead                     | 13.9                                 | 6.6                                         |
| Cadmium-silver                  | 0.4                                  | 0.0                                         |
| Used oil inspection:            |                                      |                                             |
| Visc. increase S. S. U. 100° F. | 477                                  | 251                                         |
| Naphtha insolubles              | 388                                  | 35                                          |

20 Data obtained in the same type of corrosion test with calcium oenolate alone and in combination with amyl tartrate in lubricating oil are as follows:

| 40                           | Acid treated Western oil + .5% calcium oenolate | Acid treated Western oil + .5% calcium oenolate + .2% amyl tartrate |         |
|------------------------------|-------------------------------------------------|---------------------------------------------------------------------|---------|
|                              |                                                 | 100° F.                                                             | 210° F. |
| Corrosion—wt. loss, mgs.:    |                                                 |                                                                     |         |
| Copper-lead 72 hours         | 126.4                                           | 14.0                                                                | 6.9     |
| Cadmium-silver 72 hours      | 66.1                                            |                                                                     |         |
| Used oil inspections:        |                                                 |                                                                     |         |
| Increase in visc. at 100° F. | 785                                             | 490                                                                 | 5.02    |
| Neutralization number        | 5.33                                            | 211                                                                 | 134     |
| Naphtha insolubles           |                                                 |                                                                     |         |

55 The following shows the used oil inspections of the corrosion test with calcium lanolate alone and in combination with amyl tartrate:

| 60                                             | Oil | Increase in viscosity at— |         | Neutralization number | Naphtha insolubles |
|------------------------------------------------|-----|---------------------------|---------|-----------------------|--------------------|
|                                                |     | 100° F.                   | 210° F. |                       |                    |
| Acid treated Western oil                       |     | 535                       | 13      | 3.50                  | 190                |
| Do. + .5% calcium lanolate                     |     | 365                       | 9.3     | 1.97                  | 318                |
| Do. + .2% amyl tartrate                        |     | 335                       | 13      | 3.50                  | 190                |
| Do. + .5% calcium lanolate + .2% amyl tartrate |     | 300                       | 7.4     | 1.79                  | 28                 |

65 <sup>1</sup> Values approximate.

70 In the foregoing engine tests a single cylinder, 2 5/8" bore and 2 1/2" stroke Lauson gasoline engine was operated under extremely severe conditions for the purpose of developing fully piston ring sticking and piston gumming tendencies under circumstances simulating severe operating conditions encountered in the field. Operation 75 of the motor during tests was continuous at

1600 R. P. M. speed with periodic shutdowns at fifteen-hour intervals for inspection. The jacket temperature was maintained at 375° F. and the sump oil temperature at 220° F. In the above corrosion tests the following method was utilized: Glass tubes 2" in diameter and 20" long were immersed in an oil bath, the temperature of which was automatically controlled to within  $\pm 1$ ° F. of the test temperature which was 300° F. Approximately 300 cc. of oil under test was placed in each tube and air was bubbled through it at the rate of 10 liters per hour. Strips of the two types of bearing metal were placed in the oil. In most cases the copper-lead and the cadmium-silver bearing alloys were tested simultaneously in the same sample of oil. The weight loss of each strip was recorded. Before weighing, each strip was washed in petroleum ether and carefully dried. The duration of the test was 72 hours.

It has also been discovered that hydrocarbon oils containing an inhibitor comprising a metal salt of a substituted acid of phosphorus, such as calcium cetyl phosphate, form a black deposit when contacted with metal surfaces heated to 425° F. or above. The presence of the alcoholate in an oil containing such metal phosphate salts inhibits the formation of such deposits. This property of a cooperation between the two ingredients is illustrated by a test in which a heated metal surface (hot wire) is contacted with the compounded oil at 300° F. and the temperature gradually raised to 550° F., at which point it is maintained for one hour. In this test the hot wire is partially immersed and partially exposed in air, and the amount of deposition at the oil surface is observed. The following data illustrate the improvements resulting in the above-described test:

| Oil                                                         | Deposit |
|-------------------------------------------------------------|---------|
| Acid refined Western oil S. A. E. 30.                       |         |
| Ditto + .75% calcium lanolate.                              | 0.8     |
| Ditto + .75% calcium cetyl phosphate.                       | 83.4    |
| Ditto + .5% calcium lanolate + .25% calcium cetyl phosphate | 0.0     |

An additional new result obtained by the combination of inhibitors utilized in this invention comprises increased stability of the oil solution of each of said components. Lubricating oils containing the metal phosphates alone may become cloudy in storage and the metal salts of substituted acids of phosphorus tend to precipitate from the oil solution in the presence of moisture. Some metal alcoholates are subject to precipitation from solution in lubricating oils or cloud formation in the presence of water. When both the alcoholate and the phosphate are present in the lubricating oil the solution becomes more stable against precipitation or cloud formation. Thus the metal alcoholates act as a stabilizing agent for the metal salts of the substituted acids of phosphorus and permit the preparation of more concentrated solutions of the salts than might otherwise be feasible.

From the above detailed descriptions it will be apparent that the combinations of ingredients herein disclosed give a new composition having new and highly useful properties. It is immaterial for the purpose of the present invention whether the separate components be new or old, since it is the discovery of the combination of ingredients and the unpredictable properties ob-

tained thereby which comprise applicants' contribution to the art.

The compounded lubricants herein disclosed may have one or more advantages depending upon the particular compounds selected, the proportions utilized, and the environment which the lubricating oil is to encounter. It should be observed, for example, that even though a compounded oil may be somewhat corrosive to copper-lead or cadmium-silver bearing metals, Babbitt bearings may be little if at all affected by such corrosive action. Hence, compounded oils which may not be particularly desirable for lubrication of copper-lead or cadmium-silver bearings at high temperatures where corrosion becomes a factor of importance may be highly useful and extremely advantageous in conjunction with the operation of internal combustion engines having bearings of babbitt or other corrosive-resistant bearing metals. The present invention in its broader aspects is therefore not limited to the particular combination of ingredients having all or the greatest number of advantages but embraces various of the less advantageous addition agents which will find utility in particular applications where all the possible improvements in the properties may not be required or where the standard of performance may not be so high.

A moderately acid refined naphthenic base lubricating oil is the preferred base oil stock for the compounded lubricants involved herein. The compounding ingredients appear to function more efficiently in such a base oil than in paraffinic oil stocks or highly refined naphthenic oils. However, it is to be understood that the invention is not limited to any particular base stock since advantages herein disclosed may be obtained, at least to some degree, with various oil stocks, the selection of which will be determined by conditions and service which the compounded lubricant is to encounter.

The proportion of oxidation inhibitors which may be added to mineral lubricating oils according to the principle of the present invention may vary widely depending upon the uses involved and the properties desired. As little as 0.05% by weight of various of the oxidation inhibitors gives measurable improvements. From approximately 0.1% to 2% of the compound may be added to lubricants containing metal alcoholates where stability at high temperature comprises the principal property desired. Solutions containing more than 2% of the compounds in mineral oils may be utilized for various purposes, e. g. for preparing lubricating greases and concentrates capable of dilution with lubricating oils and the like. Likewise, the proportion of metal alcoholates present in the compounded lubricant may vary widely depending upon the uses involved and the properties desired. As little as 0.1% by weight of the alcoholate gives measurable improvement, although from approximately 0.25% to approximately 2% alcoholate is preferred where the compounded oil is to be used as a crankcase lubricant for internal combustion engines. As much as 50% or more by weight of various of the alcoholates may be dissolved in mineral oil for the purpose of preparing a concentrate capable of dilution with lubricating oils and the like. Concentrates containing high percentages of the alcoholate and oxidation inhibitor comprise a convenient method of handling the ingredients and may be used

as addition agents for lubricants in general, as well as for other purposes.

The combination of ingredients of this invention may be present in hydrocarbon oils containing other compounding agents, such as pour point depressants, oiliness agents, extreme pressure addition agents, blooming agents, and compounds for enhancing the viscosity index of the hydrocarbon oil. The invention in its broader aspects embraces mineral hydrocarbon oils containing, in addition to the metal alcoholate and the oxidation inhibitor, thickening agents and/or metal soaps in grease-forming proportions or in amounts insufficient to form grease, as in the case of mineral castor machine oils or other compounded liquid lubricants.

While the character of the invention has been described in detail and numerous examples of the composition given, this has been done by way of illustration only and with the intention that no limitation should be imposed on the invention thereby. It will be apparent to those skilled in the art that numerous modifications and variations of the illustrative examples may be effected in the practice of the invention which is of the scope of the claims appended hereto.

We claim:

1. A composition of matter comprising a hydrocarbon oil, at least about 0.1% by weight based on the oil of a compound of the type formula:



where M is a metal, X is selected from the group consisting of oxygen and sulfur, C is a non-benzenoid carbon atom, R is an organic radical of hydrocarbon structure, and n may have a

value of from one to the valence of the metal; and at least about 0.05% by weight based on the oil of an organic hydroxy ester having at least one hydroxyl group not more than two carbon atoms removed from a carboxyl group of said ester.

5 2. A composition of matter comprising a hydrocarbon oil, at least about 0.1% by weight based on the oil of a compound of the type formula:



where M is a metal, X is selected from the group consisting of oxygen and sulfur, C is a non-benzenoid carbon atom, R is an organic radical of hydrocarbon structure, and n may have a value of from one to the valence of the metal; and at least about 0.05% by weight based on the oil of an organic ester of a polycarboxylic acid having two carboxyl groups no more than two carbon atoms apart.

10 3. A composition of matter comprising a hydrocarbon oil, at least about 0.1% by weight based on the oil of a compound of the type formula:



20 where M is a metal, X is selected from the group consisting of oxygen and sulfur, C is a non-benzenoid carbon atom, R is an organic radical of hydrocarbon structure, and n may have a value of from one to the valence of the metal; and at least about 0.05% by weight based on the oil of an alkaline earth organo-borate.

25

ARTHUR L. LYMAN.  
LLOYD H. MULIT.

CERTIFICATE OF CORRECTION.

Patent No. 2,341,565.

February 15, 1944.

ARTHUR L. LYMAN, ET AL.

It is hereby certified that error appears in the printed specification of the above numbered patent requiring correction as follows: Page 3, second column, line 7, for "cadmium" read --calcium--; and that the said Letters Patent should be read with this correction therein that the same may conform to the record of the case in the Patent Office.

Signed and sealed this 23rd day of May, A. D. 1944.

Leslie Frazer

(Seal)

Acting Commissioner of Patents.